

H. H. BECKWITH AND E. E. COX.

SHOE STIFFENER.

APPLICATION FILED JAN. 3, 1919.

1,391,932.

Patented Sept. 27, 1921.



Fig. 1.



Fig. 2.

Inventors  
Harry H. Beckwith,  
Edward E. Cox,  
by Wright Brown Dury, May  
Attorneys.

# UNITED STATES PATENT OFFICE.

HARRY H. BECKWITH, OF BROOKLINE, MASSACHUSETTS, AND EDWARD E. COX, OF DOVER, NEW HAMPSHIRE; SAID COX ASSIGNOR TO SAID BECKWITH.

## SHOE-STIFFENER.

1,391,932.

Specification of Letters Patent. Patented Sept. 27, 1921.

Application filed January 3, 1919. Serial No. 269,475.

To all whom it may concern:

Be it known that we, HARRY H. BECKWITH and EDWARD E. Cox, citizens of the United States, respectively residing at Brookline, in the county of Norfolk and State of Massachusetts, and at Dover, in the county of Strafford and State of New Hampshire, have invented new and useful Improvements in Shoe-Stiffeners, of which the following is 5 a specification.

This invention relates to the manufacture of materials which may be employed for various purposes in the arts, such for example, as stiffeners for the ends of footwear, etc. 10 Such materials usually comprise a foundation and a substance which will impart a certain stiffness thereto, but which under certain conditions may first be softened to permit the material to be molded or shaped, and 15 then be permitted to reset in its molded or shaped form. As illustrative of the general character of the materials referred to, it has been proposed, with commercial success, to 20 impregnate a sheet of wool felt with Montan wax or other resinous waxy asphaltic or hydrocarbon substance while the latter is in a liquid condition, and then, after the stiffening compound has hardened or set, to cut 25 from the sheets blanks of proper form to be used as box-toe or counter stiffeners. Such 30 blanks are stiff and substantially resilient, but, upon being heated to a temperature of say 160° to 180° F., become soft and limp so that they may be molded about the end 35 of a shoe last. The material which forms the subject of this specification, while capable of various uses, is however also particularly applicable for the manufacture of 40 stiffeners for box-toes and counters, and will be described in connection therewith.

Speaking generally, the invention comprises not only the new material, but also the process of producing it. The material consists of a foundation layer of any suitable character, such as a textile fabric, and a coating interlocked therewith or adherent thereto; the coating itself consisting of a mixture of fiber and a suitable, readily fusible, resinous compound, which when cold 45 imparts stiffness and relative rigidity to the foundation, but which when subjected to relatively low heat becomes soft. Any suitable disintegrated fiber may be employed such as that obtained from rags (woolen or 50 cotton), flock, or cellulose fiber, *i. e.*, ground wood, sulfite, or sulfate pulp, etc.

In practice the fiber and the stiffening compound, the latter if desired in a granular or finely comminuted condition, are thoroughly intermixed, and are spread upon the 60 foundation layer and are caused to adhere thereto or interlock therewith. This may be accomplished either by heating the mixture until the stiffening compound becomes liquid or plastic and adhesive, spreading the mixture 65 in that condition on the foundation, and pressing it thereon by pressure rolls (which may be chilled if desired), or else the mixture may, in a granular or comminuted form, be spread upon the foundation, and then 70 passed through heated rolls to soften the mixture to a plastic adhesive condition and cause it to cohere in a mass and to adhere to the foundation layer.

For making a material which may be cut 75 into blanks to be used as toe-boxes or counter stiffeners, we preferably employ as the foundation layer, burlap, on one face provided with long-fibered cotton or wool flock which mats under pressure to cover the interstices 80 in the burlap and form a smooth face. Such a foundation is preferably impregnated or saturated with a resinous compound. For this purpose, we use any suitable fusible resinous material (meaning thereby to 85 include such substances as carnauba wax, Montan wax, shellac, paraffin, copal, Kauri gums, pitch or asphalt or mixtures thereof) which may be softened or liquefied without decomposition by the application of heat. The 90 impregnating compound should be applied in a liquid condition, and to this end it may be dissolved in a suitable volatile solvent or heated to the melting point.

After the sheet of flock-faced burlap has 95 been drawn through the saturating tank and has been passed through squeeze or pressure rolls to remove the excess compound and to compact the long-fibered flock in a mat upon the face of the foundation, it is cooled or 100 dried to permit the compound to set more or less, and is then ready for the application of the coating.

The coating compound, of any of the suitable materials last referred to, may be prepared by thoroughly mixing the disintegrated fiber and the resinous compound and rendering the mass plastic and adhesive, either by the use of a solvent or by the application of heat, so that it may be spread 105 in the desired thickness upon the foundation 110 in the desired thickness upon the foundation by means of suitable machinery. After the

coating is applied, the sheet is passed through rolls, which in the case stated may be chilled or heated as desired. When the 5 coating mixture is still in a cold comminuted condition, it may be spread from a hopper upon the traveling sheet, and the sheet with the layer of the desired thickness of the mixture thereon is then passed through heated rolls which compact and heat the mixture to 10 cause it to form a cohesive mass and to interlock with and adhere to the foundation sheet. Additional calender rolls may be employed for imparting a relatively smooth glazed surface to the coating.

15 Heretofore, in the manufacture of stiffener material, a sheet of wool felt was impregnated with some one or more of the resinous materials hereinbefore referred to, and blanks were died or stamped from the 20 sheet to form the stiffener blanks of the desired shape. As already explained, because of the conformation of such blanks, there has resulted a great deal of waste material for which no commercial use has been made.

25 We have found that this waste material may be employed in preparing the coating compound for the manufacture of one embodiment of the present invention. Such waste material consists of the wool fiber (also cot-

30 ton, if the latter be used for adulterating the wool felt,) and the resinous compounds, and, when cold, is stiff and somewhat brittle. It is disintegrated and comminuted by any suitable machinery, such as a grinding machine or ball mill, while it is cold, and, after 35 it has reached the desired state of comminution and the fibers have been disintegrated, it may, while still cold, be applied to the sheet in the manner herein described, and 40 heated by the rolls to constitute a cohesive and adhering coating on the foundation.

It is highly desirable, in the manufacture 45 of shoe stiffeners, that the resinous material should not soften at moderate temperatures, that is, when exposed to blood heat or solar heat, but should soften at a temperature of say 160° to 180° F. more or less, so that, in the manufacture of the shoe containing the blank, the latter may be quickly rendered 50 soft and moldable at a temperature which will not injure leather. Hence, in making the compound to be used with the fiber, the ingredients should be so selected and compounded that they will soften at the desired 55 temperature, and set or harden rapidly to render the finished material stiff and resilient.

On the accompanying drawing, Figure 1 represents a toe-box blank embodying the invention.

Fig. 2 represents more or less conventionally a section therethrough on a large scale.

The foundation layer *a* as shown consists 65 of burlap which has on one face a mat *b* of

flock, the fibers of which are interlocked with the burlap. Such burlap is available commercially. As shown, burlap has been impregnated with a resinous compound having the characteristics herein described, and 70 the flock has been compacted into a protecting layer on one face thereof. On the other face, there is a layer *c* consisting of fiber and resinous stiffening compound, such as herein described. The blank which is illustrated is for stiffening the box-toe of a shoe, and it has been skived along the edge as at *d*. Of course, if desired, the coating may be applied to both faces of the foundation sheet.

Having thus explained the nature of our said invention and described a way of making and using the same, although without attempting to set forth all of the forms in which it may be made or all of the modes of 85 its use, what we claim is:

1. A stiff resilient sheet comprising a foundation of flexible woven fibrous material and a coating adherent on the face thereof and interlocked therewith, said coating consisting of a mixture of disintegrated fiber and a resinous compound which is stiff and hard when cold but is capable of being softened, and then setting in a rigid state.

2. A stiff resilient shoe stiffener blank 95 comprising a foundation of flexible woven fibrous material and a stiffening coating, said coating consisting of a mixture of disintegrated fiber and a fusible resinous compound capable of being softened by the application of heat.

3. A stiff resilient shoe stiffener blank comprising a textile foundation saturated with a resinous body, and a coating consisting of an adherent layer of disintegrated fiber and a resinous compound in admixture, and capable of being softened and then setting, whereby said blank may be molded on the end of a last.

4. A resilient shoe stiffener blank comprising a foundation of burlap and a coating thereon consisting of a mixture of disintegrated fiber and a resinous compound, said coating rendering said foundation stiff but being capable of softening upon the application of heat, so that said blank may be molded into form and then permitted to set.

5. A stiffener blank comprising a foundation consisting of flock faced textile material impregnated with a resinous compound and having the flock matted upon the face thereof, and a coating interlocked with the other face thereof and consisting of a mixture of disintegrated fiber and a binder adapted to be softened by heat.

In testimony whereof we have affixed our signatures.

HARRY H. BECKWITH.  
EDWARD E. COX.